

## UNITED STATES PATENT OFFICE

EARL H. BUNCE AND THOMAS C. ROUTSON, OF PALMERTON, PENNSYLVANIA, ASSIGNEES  
TO THE NEW JERSEY ZINC COMPANY, OF NEW YORK, N. Y., A CORPORATION OF NEW  
JERSEY

## PREPARING COKE AGGLOMERATES

No Drawing.

Application filed August 23, 1928. Serial No. 301,709.

This invention relates to the reduction of zinciferous material and is more especially concerned with that method of reduction in which the charge consists of coked agglomerates of mixed zinciferous material and carbonaceous material. The invention aims to provide certain improvements in the preparation of such coked agglomerates.

It has heretofore been found that coked agglomerates of mixed zinciferous and carbonaceous materials constitute a peculiarly advantageous charge for vertical zinc distillation retorts. Such agglomerates must not split up during coking and must possess sufficient residue strength, i. e., sufficient strength to pass progressively through the vertical retort without breaking down or sanding, thereby preserving throughout the entire reducing operation that desirable uniform porosity of the charge which enables economic and efficient transfer of heat by hot gases from the hot wall of the retort to the center or core of the charge, and permitting the free passage of the zinc vapor and the gases through the vertical retort to their place of exit.

These agglomerates are prepared by first crushing the ore and coal separately, then kneading them together, in a Chilean mill or edge-runner to form a mixture that is suitable for agglomerating. The Chilean mill or edge-runner is frequently referred to as a "chaser", its operation as "chasing", and the treated material as having been "chased". A binder, if necessary, such as sulfite liquor, may be added in the last stage of the treatment in the edge-runner. The mixture thus prepared in the edge-runner is then agglomerated and coked, at temperatures insufficient to cause any substantial loss of zinc.

We have found that certain details of the preparation of the mixture of coal and zinc ore or the like before agglomerating influence to a marked extent the ultimate properties of the coked agglomerates, and the essential nature of the present invention relates to a control of the preparation of the zinc ore and the coal before agglomerating, in such a manner as to secure the production of agglomerates that will not split up when coked

and that will not disintegrate when smelted in a vertical retort for the distillation of zinc.

The appropriate control of the preparation of the charge for agglomeration involves a proper adjustment of at least the following three factors: (1) nature of the coal, with particular reference to its coking characteristics; (2) particle size of (a) the zinc ore and (b) the coal, before they are kneaded together in the edge-runner; (3) particle size of the mixture of zinc ore and coal, after treatment in the edge-runner, in the final stage of its preparation for agglomeration. These three factors may be appropriately controlled in combination, to secure a firm agglomerate consisting of a coke structure intimately bonded with and enveloping the particles of zinc ore, so as to prevent both splitting up of the agglomerates during coking and disintegration during the subsequent distillation.

We have found that the carbonaceous material used to prepare the agglomerates should be composed in part of a so-called "free-flowing" coal, i. e., a coal that during coking softens to a great extent, wetting the individual particles of ore, so that when the coke hardens substantially each ore particle is enveloped in and in intimate contact with coke; and, when the ore particles are later disintegrated by the expulsion of their zinc content during the distillation the gaps left in the structure are as small as possible, so that the strength of the residue is preserved. However, such free-flowing coals as a rule swell or puff up when heated to coking temperatures, and are then known as swelling coals. This property of swelling is undesirable in the preparation of coked agglomerates of zinc ore and coal, since the swelling tends to split up the agglomerates during the coking operation. This tendency of the swelling free-flowing coal to split up the briquettes is, according to the present invention, overcome by appropriate blending with a coal that does not swell during coking. This non-swelling coal need not necessarily be free-flowing; indeed, even non-coking carbonaceous material, such as anthracite coal dust

and coke breeze or the like may advantageously form part of the blend.

In practice, we find that the uncoked agglomerate mixture may advantageously contain around 15%, by weight, of a free-flowing and swelling coal of high coking quality, but that the amount of such swelling coal used should not exceed 20-25% by weight on the agglomerate mixture before coking.

- 10 Coal of bituminous rank mined from the Pittsburg seam of the Monongahela series in the Preston-Taylor mining district, Taylor County, West Virginia, is a high volatile free-flowing and swelling coal of excellent coking quality. Agglomerate mixtures of about 50% roasted zinc flotation concentrates and 50% of this coal, when briquetted and coked, flow and swell during coking, and the resulting coked agglomerates stick together and are objectionably distorted and ruptured, although of very satisfactory strength. By appropriately blending the above-described free-flowing and swelling coal with a non-swelling or shrinking coal, 25 a very satisfactory carbonaceous mixture for coked agglomerates may be produced. Thus, with the 50-50 mixture of ore and reduction fuel, we have secured satisfactory results with a blend of from 20-10% of the above- 30 mentioned free-flowing and swelling coal and from 30-40% of coal of bituminous rank mined from the Pittsburg seam of the Monongahela series in the Connellsville mining district, Fayette County, Pennsylvania, 35 a very slightly swelling coal of good coking quality. This blend is further improved by substituting anthracite coal dust, coke breeze, or similar non-coking carbonaceous material, for a small percentage of the coking 40 coals. Thus, we have secured excellent results with the following agglomerate mixture.

|                         | Per cent<br>by weight |
|-------------------------|-----------------------|
| 45 Zinciferous material | 55.5                  |
| Preston-Taylor coal     | 18.5                  |
| Connellsville coal      | 18.5                  |
| Anthracite dust coal    | 7.5                   |

- 50 As a representative standard for an agglomerate mixture of 60 parts of zinciferous material and 40 parts of carbonaceous material, we have found the following proportions one of general application:

|                                          | Per cent<br>by weight |
|------------------------------------------|-----------------------|
| 55 Zinciferous material                  | 60                    |
| Free-flowing coal of good coking quality | 15                    |
| Non-swelling coal of good coking quality | 25                    |

- 60 Where the free-flowing coking coal tends to swell during coking, the inclusion of a small amount of anthracite coal or coke breeze serves to dampen this tendency. Thus, we have found that certain lots of 65 Tower Hill coal evidence this tendency to

swell, and in such cases we have secured satisfactory results with the following mixture:

|                                     | Per cent<br>by weight |
|-------------------------------------|-----------------------|
| Roasted zinc flotation concentrates | 61.5                  |
| Preston-Taylor coal                 | 11.5                  |
| Connellsville coal                  | 19                    |
| Anthracite dust coal                | 8                     |

We have furthermore secured satisfactory results with the following blend of a swelling coal of good coking quality and anthracite dust coal:

|                                    | Per cent<br>by weight |
|------------------------------------|-----------------------|
| Roasted zinc flotation concentrate | 60                    |
| Preston-Taylor coal                | 30                    |
| Anthracite dust coal               | 10                    |

The anthracite dust coal in these mixes serves to maintain the coke structure and give residue strength during the zinc distillation operation. Crushed coke, coke breeze, and similar non-coking carbonaceous materials may be substituted for the anthracite dust coal.

The particle size of both the ore and the coal affects the intimacy of contact of the ore and coal brought about by the subsequent treatment in the edge-runner, as well as the capacity of compacting thus brought about.

Optimum results appear to be secured when the bituminous coking coal is of a graded size with not more than about 16% on a 14 mesh screen and not more than about 16% through a 200 mesh screen, the remaining 68% displaying a substantially uniform gradation of size. The following data may be considered for illustrative purposes:

Table No. I

| Bituminous coal         | %    | Hammer mill<br>crushed cu-<br>mulative % |
|-------------------------|------|------------------------------------------|
| On 8 mesh screen        | 4.3  | 95.7                                     |
| 14 mesh screen          | 11.8 | 83.9                                     |
| 20 mesh screen          | 10.6 | 73.3                                     |
| 28 mesh screen          | 9.6  | 63.7                                     |
| 35 mesh screen          | 11.3 | 51.9                                     |
| 48 mesh screen          | 8.9  | 43.0                                     |
| 65 mesh screen          | 7.5  | 35.5                                     |
| 80 mesh screen          | 3.6  | 31.9                                     |
| 100 mesh screen         | 4.6  | 27.3                                     |
| 150 mesh screen         | 5.8  | 21.5                                     |
| 200 mesh screen         | 5.0  | 16.5                                     |
| Through 200 mesh screen | 16.5 |                                          |

It is desirable, but not necessary, that the non-coking carbonaceous material of the agglomerate mixture be of the aforementioned graded particle size, and the closer this is approximated the more closely will the coked agglomerates approximate the optimum desired properties. We have, however, successfully used for the non-coking carbonaceous material of the foregoing mixes coke crushed to pass through 8 mesh.

Optimum results appear to be secured when the zinc ore, if roasted, is of a graded size with not more than about 4.0% on a 14 mesh screen and not more than about 38% through

a 200 mesh screen, the remaining 58% displaying a continuous gradation of size, with gradual increase in the weight of material through the finer screens. The following data may also be considered for illustrative purposes:

Table No. II

|    | Roasted flotation concentrates | %    | % cumulative |
|----|--------------------------------|------|--------------|
| 10 | On 8 mesh screen               | 1.9  | through 98.1 |
|    | 14 mesh screen                 | 1.3  | 96.8         |
|    | 20 mesh screen                 | 0.7  | 96.1         |
|    | 28 mesh screen                 | 0.5  | 95.6         |
|    | 35 mesh screen                 | 0.9  | 94.7         |
|    | 48 mesh screen                 | 1.3  | 93.4         |
|    | 65 mesh screen                 | 2.8  | 90.6         |
|    | 80 mesh screen                 | 4.1  | 86.5         |
|    | 100 mesh screen                | 10.9 | 75.6         |
| 15 | 150 mesh screen                | 18.9 | 56.7         |
|    | 200 mesh screen                | 19.3 | 37.4         |
|    | Through 200 mesh screen        | 37.4 |              |

In the case of unroasted zinc ores, such as zinc silicate (willemite), it appears that the particles may be substantially coarser, as indicated by the following illustrative data:

Table No. III

|    | Unroasted zinc silicate willemite ore | %    | % cumulative |
|----|---------------------------------------|------|--------------|
| 25 | On 8 mesh screen                      | 0    | through 100  |
|    | 14 mesh screen                        | 0    | 100          |
|    | 20 mesh screen                        | .1   | 99.9         |
|    | 28 mesh screen                        | .3   | 99.6         |
|    | 35 mesh screen                        | 6.6  | 93.0         |
|    | 48 mesh screen                        | 16.9 | 76.1         |
| 30 | 65 mesh screen                        | 24.4 | 51.7         |
|    | 80 mesh screen                        | 9.4  | 42.3         |
|    | 100 mesh screen                       | 13.2 | 29.1         |
|    | 150 mesh screen                       | 14.0 | 15.1         |
|    | 200 mesh screen                       | 9.2  | 5.9          |
|    | Through 200 mesh screen               | 5.9  |              |

The particle size of the mixture of ore and coal after treatment in the edge-runner is also of importance. The chased material should have a particle size that is consistent with the formation of an agglomerate of optimum or at least adequate coking and residue strengths. Thus, if the particle size of the chased material is too fine, the agglomerates will be relatively dense and compact. During the subsequent coking and/or reduction operations, the volatile constituents will escape from the agglomerate with extreme difficulty, if at all. In order to drive the volatile hydrocarbons and zinc from the agglomerate, considerable pressure will be set up within the agglomerate. Stresses and strains take place within and the agglomerate will usually rupture and disintegrate. Such a result works away from porosity of the charge, is therefore harmful, and should be avoided.

On the other hand, if the particle size of the chased material is too coarse, the agglomerates will not be as dense and compact as they should be to insure adequate, let alone optimum, coking and residue strengths. In other words, there appears to be a happy mean of particle size for the chased material which is compatible with the formation of an agglomerate that will have adequate or optimum coking and residue strengths. The following tables give data that may be regarded as illustrative of this point, as par-

ticularly observed with respect to certain mixtures of zinc ore and coals:

Table IV

|  | Chased mix consisting of:         |                        |                    |    |
|--|-----------------------------------|------------------------|--------------------|----|
|  | 60 roasted flotation concentrates | 30 Preston-Taylor coal | 10 anthracite coal | 70 |
|  | On 8 mesh screen                  | % on                   | % on               |    |
|  | 14 mesh screen                    | 4.9                    | 93.9               |    |
|  | 20 mesh screen                    | 4.5                    | 89.4               |    |
|  | 28 mesh screen                    | 3.8                    | 85.6               |    |
|  | 35 mesh screen                    | 5.1                    | 80.5               | 75 |
|  | 48 mesh screen                    | 3.5                    | 77.0               |    |
|  | 65 mesh screen                    | 3.4                    | 73.6               |    |
|  | 80 mesh screen                    | 1.8                    | 71.8               |    |
|  | 100 mesh screen                   | 2.2                    | 69.6               |    |
|  | 150 mesh screen                   | 4.0                    | 65.6               |    |
|  | 200 mesh screen                   | 4.8                    | 60.8               |    |
|  | Through 200 mesh screen           | 60.8                   |                    | 80 |

Table V

|  | Chased mix consisting of:         |                                     |                                       |    |
|--|-----------------------------------|-------------------------------------|---------------------------------------|----|
|  | 50 roasted flotation concentrates | 20 Preston-Taylor free flowing coal | 30 Connellsville slight swelling coal | 85 |
|  | On 8 mesh screen                  | % on                                | % on                                  |    |
|  | 14 mesh screen                    | 3.4                                 | 96.0                                  |    |
|  | 20 mesh screen                    | 5.8                                 | 90.2                                  |    |
|  | 28 mesh screen                    | 5.7                                 | 84.5                                  |    |
|  | 35 mesh screen                    | 7.6                                 | 76.9                                  |    |
|  | 48 mesh screen                    | 6.9                                 | 70                                    |    |
|  | 65 mesh screen                    | 8.6                                 | 61.4                                  | 90 |
|  | 80 mesh screen                    | 5.2                                 | 56.2                                  |    |
|  | 100 mesh screen                   | 6.1                                 | 50.1                                  |    |
|  | 150 mesh screen                   | 8.4                                 | 41.7                                  |    |
|  | 200 mesh screen                   | 6.6                                 | 35.1                                  |    |
|  | Through 200 mesh screen           | 35.1                                |                                       |    |

Table VI

|  | Chased mix consisting of:           |                                  |                          |     |
|--|-------------------------------------|----------------------------------|--------------------------|-----|
|  | 61.5 roasted flotation concentrates | 11.5 Preston-Taylor free flowing | 8.0 anthracite dust coal | 95  |
|  | On 8 mesh screen                    | % on                             | % on                     |     |
|  | 14 mesh screen                      | 4                                | through 99.6             |     |
|  | 20 mesh screen                      | 2.0                              | 97.6                     | 103 |
|  | 28 mesh screen                      | 2.5                              | 95.1                     |     |
|  | 35 mesh screen                      | 2.2                              | 92.9                     |     |
|  | 48 mesh screen                      | 3.8                              | 89.1                     |     |
|  | 65 mesh screen                      | 3.1                              | 86.0                     |     |
|  | 80 mesh screen                      | 3.0                              | 83.0                     |     |
|  | 100 mesh screen                     | 2.7                              | 81.0                     |     |
|  | 150 mesh screen                     | 5.6                              | 78.3                     | 105 |
|  | 200 mesh screen                     | 5.6                              | 72.7                     |     |
|  | Through 200 mesh screen             | 67.1                             | 67.1                     |     |

Table VII

|  | Chased mix consisting of: |                         |                                                  |     |
|--|---------------------------|-------------------------|--------------------------------------------------|-----|
|  | 60 unroasted silicate ore | 20 anthracite dust coal | 20 Preston-Taylor free flowing and swelling coal | 110 |
|  | On 8 mesh screen          | % on                    | % on                                             |     |
|  | 14 mesh screen            | 2.2                     | 99.5                                             |     |
|  | 20 mesh screen            | 3.1                     | 97.3                                             |     |
|  | 28 mesh screen            | 2.9                     | 94.2                                             |     |
|  | 35 mesh screen            | 5.7                     | 91.3                                             |     |
|  | 48 mesh screen            | 8.1                     | 85.6                                             |     |
|  | 65 mesh screen            | 11.3                    | 77.5                                             |     |
|  | 80 mesh screen            | 5.4                     | 66.2                                             |     |
|  | 100 mesh screen           | 7.9                     | 60.8                                             |     |
|  | 150 mesh screen           | 10.8                    | 52.9                                             | 115 |
|  | 200 mesh screen           | 8.5                     | 42.1                                             |     |
|  | Through 200 mesh screen   | 33.6                    | 33.6                                             |     |

The graded particle size of the ingredients of the agglomerate mixture, contemplated by the present invention, insures such density of the mixture as will give adequate if not maximum strength of the coked agglomerate. This graded particle size furthermore promotes the desired intimate mixture of the zinciferous and carbonaceous materials and insures better compacting of these materials by briquetting, extrusion and like operations. 120 125 130

Where the agglomerate mixture is too dense, cracking or rupturing of the agglomerates is liable to take place during the coking operation, and if the mixture is not dense enough the coked agglomerates are deficient in strength, particularly in residue strength during the subsequent reduction operation. The graded particle sizes herein contemplated produce a mixture of adequate or optimum density with respect to the desired ultimate properties of the coked agglomerates.

The agglomerate mixtures for zinc distillation are usually made up from 35 to 65% by weight of zinciferous material and from 15 to 35% by weight of carbonaceous material. In general, the higher the zinc content and the more finely divided the zinciferous material, the more coal will be needed in the mixture. The examples given above illustrate the manner in which the proportions of coals may be suitably blended when worked with certain zinciferous materials, and the relation of the total coal content to the ore, in order to secure very favorable results. It will, of course, be understood that the examples and tables given above are to be regarded as illustrative, rather than restrictive, of the invention. It is altogether possible that some variations of the figures herein referred to are necessary to secure optimum results under other and varied circumstances, such as in the type of coals and/or ores employed. The principles of the present invention are, however, applicable in such situations.

The chased material is then suitably agglomerated. For this purpose it may be advisable to use a binder in appropriate amounts. The agglomerates may be formed in various sizes and shapes and with varying degrees of density and compactness. Such factors as size, shape and density of the agglomerates will be largely governed by the particular coking and reduction operations to be employed. Other conditions being equal, the longer the column of agglomerates placed in a coking and in a reduction retort, the stronger should be the agglomerates near the bottom of the column to avoid breaking down by compressive forces. Any suitable apparatus may be employed for both the coking and reduction operations. In the present preferred practice of the invention, the agglomerates are coked by direct heating and the coked agglomerates are then melted for the recovery of their zinc content in an externally heated vertical retort.

We claim:

1. The method of preparing coked agglomerates of zinciferous material and carbonaceous material which comprises intimately mixing the zinciferous material with the carbonaceous material, the carbonaceous material containing from 15 to 25% by weight with respect to the total weight of the mixture of a free-flowing and swelling coal of

good coking quality, forming the resulting mixture by pressure into agglomerates, and subjecting the agglomerates to a coking operation.

2. The method of preparing coked agglomerates of zinciferous material and carbonaceous material which comprises intimately mixing from 35 to 65% by weight of the zinciferous material with from 65 to 35% by weight of carbonaceous material, the carbonaceous material being made up of from 15 to 25% by weight with respect to the total weight of the mixture of a free-flowing and swelling coal of good coking quality, forming the resulting mixture by pressure into agglomerates, and subjecting the agglomerates to a coking operation.

3. The method of preparing coked agglomerates of zinciferous material and carbonaceous material which comprises intimately mixing the zinciferous material with the carbonaceous material, the carbonaceous material being made up of a mixture of a free-flowing and swelling coal of good coking quality and the balance of a substantially non-swelling coal, forming the resulting mixture by pressure into agglomerates, and subjecting the agglomerates to a coking operation.

4. The method of preparing coked agglomerates of zinciferous material and carbonaceous material which comprises intimately mixing the zinciferous material with the carbonaceous material, the carbonaceous material being made up of a blended mixture of coking coals, consisting of free-flowing-swelling and slightly swelling coals, forming the resulting mixture by pressure into agglomerates, and subjecting the agglomerates to a coking operation.

5. The method of preparing coked agglomerates of zinciferous material and carbonaceous material which comprises intimately mixing the zinciferous material with the carbonaceous material, the carbonaceous material being made up of a blended mixture of coals that will be substantially non-swelling consisting of free-flowing-swelling, swelling and non-swelling coals of good coking quality, forming the resulting mixture by pressure into agglomerates and subjecting the agglomerates to a coking operation.

6. The method of preparing coked agglomerates of zinciferous material and carbonaceous material which comprises intimately mixing the zinciferous material with the carbonaceous material, the carbonaceous material being made up of from 15 to 25% by weight with respect to the total weight of the mixture of a free-flowing and swelling coal of good coking quality and the balance of a non-coking carbonaceous material, forming the resulting mixture by pressure into agglomerates, and subjecting the agglomerates to a coking operation.

7. The method of preparing coked agglom-

erates of zinciferous material and carbonaceous material which comprises intimately mixing the zinciferous material with the carbonaceous material, the carbonaceous material being made up of about equal parts by weight of a free-flowing and swelling coal of good coking quality and a non-coking carbonaceous material, forming the resulting mixture by pressure into agglomerates, and 10 subjecting the agglomerates to a coking operation.

8. The method of preparing coked agglomerates of zinciferous material and carbonaceous material which comprises intimately mixing the zinciferous material with a blended carbonaceous material containing substantial proportions of a free-flowing and swelling coal of good coking quality and a non-coking carbonaceous material, forming 20 the resulting mixture by pressure into agglomerates, and subjecting the agglomerates to a coking operation.

9. The method of preparing coked agglomerates of zinciferous material and carbonaceous material which comprises intimately mixing the zinciferous material with carbonaceous material made up in large part of a free-flowing and swelling coal of good coking quality of such particle size that not 30 more than about 16% is on 14 mesh and not more than about 16% is through 200 mesh, forming the resulting mixture by pressure into agglomerates, and subjecting the agglomerates to a coking operation.

35 10. The method of preparing coked agglomerates of zinciferous material and carbonaceous material which comprises intimately mixing the zinciferous material with carbonaceous material made up in large part 40 of a free-flowing coal of good coking quality of such particle size that at least 50% by weight is graded between 20 and 100 mesh and not more than about 16% by weight is through 200 mesh, forming the resulting mixture 45 by pressure into agglomerates, and subjecting the agglomerates to a coking operation.

11. The method of preparing coked agglomerates of zinciferous material and carbonaceous material which comprises intimately mixing the zinciferous material with carbonaceous material, said carbonaceous material consisting in part of bituminous free-flowing and swelling coal of a particle 55 size adapted to give a screen analysis of not more than about 16% on a 14 mesh screen and not more than about 16% through a 200 mesh screen, the material passing through a 14 mesh screen and remaining on a 200 mesh screen displaying a substantially uniform gradation of size, and in part of a non-swelling coal adapted to off-set the swelling effects 60 of said free-flowing and swelling coal, forming the resulting mixture by pressure into 65

agglomerates, and subjecting the agglomerates to a coking operation.

12. The method of preparing coked agglomerates of zinciferous material and carbonaceous material which comprises intimately mixing the zinciferous material with carbonaceous material, said carbonaceous material consisting of a blended mixture of coals adapted to give a good coking effect without substantial swelling, said zinciferous material consisting of roasted zinc ore of a particle size adapted to give a screen analysis of not more than about 4% on a 14 mesh screen and not more than about 38% through a 200 mesh screen, the material passing 70 through a 14 mesh screen and remaining on a 200 mesh screen displaying a substantially uniform gradation of size, forming the resulting mixture by pressure into agglomerates, and subjecting the agglomerates to a 75 coking operation.

13. The method of preparing coked agglomerates of zinciferous material and carbonaceous material which comprises intimately mixing the zinciferous material with carbonaceous material, said carbonaceous material consisting in part of bituminous free-flowing and swelling coal of a particle size adapted to give a screen analysis of not more than about 16% on a 14 mesh screen and not more than about 16% through a 200 mesh screen, the material passing 80 through a 14 mesh screen and remaining on a 200 mesh screen displaying a substantially uniform gradation of size, and in part of a non-swelling coal adapted to off-set the swelling effects of said free-flowing and swelling coal, said zinciferous material consisting of roasted zinc ore of a particle size adapted to give a screen analysis of not more than about 4% on a 14 mesh screen and not more than about 38% through a 200 mesh screen, the remaining 85 90 displaying a substantially uniform gradation of size, forming the resulting mixture by pressure into agglomerates, and subjecting the agglomerates to a coking operation.

14. The method of preparing coked agglomerates of zinciferous material and carbonaceous material which comprises intimately mixing the zinciferous material with blended carbonaceous material adapted to yield a mass of good coking but substantially non-swelling qualities, kneading and grinding together said material until the resulting mixture is composed of particles adapted to give a screen analysis of not more than about 10% on a 14 mesh screen and not more than about 70% through a 200 mesh screen, forming the resulting mixture by pressure into 100 agglomerates, and subjecting the agglomerates to a coking operation.

15. The method of preparing coked agglomerates of zinciferous material and carbonaceous material which comprises inti- 105 110 115 120 125 130

mately mixing the zinciferous material with carbonaceous material, said carbonaceous material consisting in part of bituminous free-flowing and swelling coal of a particle size adapted to give a screen analysis of not more than about 16% on a 14 mesh screen and not more than about 16% through a 200 mesh screen, the material passing through a 14 mesh screen and remaining on a 200 mesh screen displaying a substantially uniform gradation of size, and in part of a non-swelling coal adapted to off-set the swelling effects of said free-flowing and swelling coal, said zinciferous material consisting of roasted zinc ore of a particle size adapted to give a screen analysis of not more than about 4% on a 14 mesh screen and not more than about 38% through a 200 mesh screen, the material passing through a 14 mesh screen and remaining on a 200 mesh screen displaying a substantially uniform gradation of size, kneading and grinding together said materials until the resulting mixture is composed of particles adapted to give a screen analysis of not more than about 10% on a 14 mesh screen and not more than about 70% through a 200 mesh screen, forming the resulting mixture by pressure into agglomerates, and subjecting the agglomerates to a coking operation.

In testimony whereof we affix our signatures.

EARL H. BUNCE.  
THOMAS C. ROUTSON.

35

40

45

50

55

60

65